

March 25, 1952

D. S. GROVE

2,590,697

ENDLESS ABRASIVE BELT AND METHOD OF MANUFACTURING SAME

Filed April 8, 1949



FIG. 1.



FIG. 2.



FIG. 4.

FIG. 6.



FIG. 5.



INVENTOR.  
DON S. GROVE,

*Allen & Allen*

ATTORNEYS.

## UNITED STATES PATENT OFFICE

2,590,697

ENDLESS ABRASIVE BELT AND METHOD OF  
MANUFACTURING SAME

Don S. Grove, Carnegie, Pa.

Application April 8, 1949, Serial No. 86,184

12 Claims. (Cl. 51—297)

1

This invention relates to an endless abrasive belt and methods for manufacturing the same. While belts according to my invention are of general utility, they have been developed particularly for use in the grinding of steel strip, sheets and bars, preliminary to coiling the strip into coils, or finishing operations on sheets and bars. Heretofore, in the grinding and polishing of coils, sheets and bars the abrasive belts used have been of paper. Paper belts, however, are subject to many disadvantages in connection with their use for grinding of steel strip, sheets and bars. In the grinding of strip, sheets and bars a tremendous amount of heat is generated and the temperature of the belt may reach 250° F. or more at the point of contact. This high heat has a deleterious effect on paper belts, in that it causes separation of the paper plies which are secured together with a glutinous adhesive which softens and fails under the influence of heat and continuous flexing. Furthermore, paper belts are adversely affected by various of the polishing oils which are presently used as lubricants, and which weaken the splice and fibers of the paper. Paper belts are, of course, hygroscopic, and are subject to changes in atmospheric conditions so that the length of the belt changes with atmospheric conditions. The expansion and contraction with changes in relative humidity cause breakage of the paper and reduce the effectiveness of the adhesive used to secure the abrasive grains to the belt.

In paper belts, if there happens to be a line burr along the edge of the strip, sheet or bar, resulting from a slitting or shearing operation, instead of the abrasive belt grinding down the burr, the burr will most often cut the paper, and as soon as the paper is torn it is useless and the belt must be scrapped. The same result will follow from strip, sheets or bars having cracked edges, or the like. The changing of belts in mid-coil necessitates stopping the entire production line, while belts are being changed, and the change time has been found to be unduly high.

It has been found that strip, sheet and bar stock characterized by camber, cross-bar or a buckled condition, cannot be ground with paper belts because the excessive, highly localized pressures cause the belt to break, tear or wrinkle, so that it has to be scrapped. For these reasons the replacement cost of belts has been unnecessarily high and of course has resulted in a higher cost per ton of finished material.

With the foregoing considerations in mind it is an object of my invention to provide a belt which will be of greatly increased strength, and

which will therefore not disintegrate by reason of having to grind down burrs or rough edges on the strip, sheet or bars.

It is another object of my invention to provide 5 a belt which is completely moistureproof, so that it will not be affected by atmospheric conditions.

It is still another object of my invention to provide a belt of such durability that when the 10 abrasive material is worn down the belt can be recoated and re-used numerous times, say, as many as 600 times.

It is yet another object of my invention to provide 15 a belt which will be of constant thickness throughout its length whereby the quality of the ground and polished strip, sheet or bars, will be enhanced.

A further object of my invention resides in the provision of a belt for fine finishing operations, which will operate without chatter. I have found 20 that chatter is caused by a hinging action at the belt joint, and therefore this object of my invention involves the provision of a helically wound belt, whereby chatter is eliminated.

Another object of my invention involves the 25 provision of a method for manufacturing a belt as outlined above whereby other of the objects discussed above are achieved. This last mentioned object includes the object of providing a new method of applying abrasive grains to the 30 belt in a manner which will render the belt more satisfactory, and give it a longer useful life for each coating.

These and other objects of the invention which 35 will become apparent to one familiar with the art upon study of these specifications, I accomplish by that certain construction and arrangement of parts, and by that series of method steps, of which I shall now disclose exemplary embodiments.

40 Reference is made to the drawings forming a part hereof, and in which:

Figure 1 is a fragmentary plan view of a belt according to my invention with parts broken away;

45 Figure 2 is a longitudinal cross-sectional view of the same with the plies separated in part to show the construction;

Figure 3 is a side elevational view of a machine suitable for the application of the abrasive coating;

50 Figure 4 is a plan view of the same taken on the line 4—4 of Figure 3;

Figure 5 is a fragmentary cross-sectional view on a greatly enlarged scale of a finished belt, 55 and

Figure 6 is a more or less diagrammatic view

2

of another way in which belts may be assembled.

The belt according to my invention is of two or more plies. The plies themselves are of textile material preferably of a material chosen from the group consisting of cotton rayon, nylon and ramie. This textile material will have a weight per square yard between three ounces and thirty-eight ounces, or even more. The particular weight of material is selected to meet the particular conditions as to light or heavy duty to which the belt is to be subjected.

That ply which is to be the outside in the finished belt is coated on its underside with an elastomer. This elastomer may be that known as Neoprene, which is made by polymerizing chlorobutadiene under pressure. All the remaining plies are impregnated with an elastomer such as Neoprene by being immersed in the elastomer and having the excess material knifed off. The weight of the drying solids based on the weight of the textile material will be in the range from about 40% to about 95%, but preferably in the vicinity of 70%. After impregnation and coating the plies are dried to drive off the solvent in the impregnating material by being drawn through a heated chamber at a temperature of about 200° F. It will be observed from the foregoing that all the plies but one are impregnated with the elastomer, while the one ply is coated on one side only with the elastomer. The uncoated side of said one ply will be the side to which the abrasive grains are applied in the finished belt.

The various plies are then passed over a steam heated table, or the like, to soften the elastomer with which they are coated or impregnated. The plies are plied together and adhesively bonded to each other with a latex adhesive in such manner that the untreated sides of said one ply is on the outside. The laminated plies are then calendered to stretch and finish the belt. The calendered belt is then vulcanized in a rotative press or the like at a pressure of about 2,000 pounds per square inch and at a temperature of about 325° F.

A belt assembled as described above will have its plies thoroughly and tightly bonded to each other, and I have determined that the adhesive strength between plies will be between 40 and 55 pounds per square inch per ply after the belt has been permitted to cool.

It will be understood that up to this point the plies have been treated in considerable width. At this stage of the process the belt edges are cut square to the desired width of the finished belt, and the cut edges have then applied to them an elastomer to protect them and to seal them. This elastomer may again be Neoprene and may, if desired, be pigmented.

The belt treated as above described is then cut to the desired length. The ends of the belt are cut so that the ends of the plies are stepped and so that the ends of the plies are on a bias at an angle to the belt edge. In this way, when the belt is finally assembled into endless form, the bias ends of the individual plies are in abutting relation with the butt joints of the respective plies in stepped relation lengthwise of the belt. This construction may be understood with reference to Figures 1 and 2 in which the respective plies are indicated at 10, 11 and 12. The solid line at 13 indicates the butt joint between the two ends of the ply 10. The butt joint between the plies 11 is indicated by the broken line at 14, and the butt joint between the ends of the ply 12 is

indicated by the broken line 15. As seen in Figure 2, the ply 15 and the ply 14 have been impregnated with the elastomer, while the ply 10 has only been coated on its under side with the elastomer. Each of the inner surfaces of the plies has been coated with the latex adhesive as indicated at 16, and the upper surface of the ply 10 is untreated.

The joint as described above is then again vulcanized in a lap press having steam heated platens at a temperature of about 325° F. In this way a smooth even joint of constant thickness is insured.

I have indicated more or less diagrammatically in Figure 6, another way in which the plies may be assembled. As there shown, one ply comprising a long strip of relatively narrow material is wound spirally upon a mandrel, as indicated by the broken lines 17. The outer ply of similar material is wound over the plies 17 in the opposite direction, as indicated by the solid lines 18. The plies themselves will have been treated as described above. When a belt has been assembled according to Figure 6 it may be removed from the mandrel and used in its then form. If desired, of course, a belt of considerable width may be manufactured according to the diagram of Figure 6, and the belt may then be slit into desired widths.

30 The belt is now ready for the application of the abrasive grains. The abrasive material used may be aluminum oxide grains, silicon carbide grains, garnet, emery, or any other suitable abrasive grains. The machine shown in Figures 3 and 4 is somewhat diagrammatic, but it comprises, for example, two fixed rolls 19 and 20 over which the belt passes, one of which rolls may be driven, as indicated by the belt and pulley 21, seen in Figure 4. A third roll 22 is preferably provided on a pivoted arm 23 so that the tension on the belt may be adjusted, and also to facilitate placing the belt on the machine and removing it from the machine. The various pulleys are suitably mounted on a frame indicated generally at 24, and between the pulleys 19 and 20 a supporting plate 25 is provided.

45 The adhesive is applied to the belt by means of a hopper 26 having a spout 27. The spout 27 of course extends entirely across the width of the belt to be treated, and conventional means for controlling the flow of adhesive from the hopper may be provided. The thickness of the adhesive coating, and its thorough distribution (particularly where a previously used belt having residual grains on its surface is to be recoated, and where it is important that the adhesive enters into the interstices between grains) are insured by the calender roll 27a, and the excess adhesive is scraped off by a doctor blade 27b. 50 The calender roll 27a should be quite soft to accomplish the purpose, and therefore an elastomer such as Neoprene of 25 Durometer hardness is about the hardest that can be used. It is much preferred to use an elastomer such as Neoprene of about 15 Durometer hardness. Means (not shown) are provided for imparting to the calender roll 27a a reciprocating movement transversely of the belt, as well as an oscillating movement in a plane parallel to the belt. The adhesive is preferably of the sodium silicate type, but it may be magnesium oxychloride, or other suitable adhesive. While the adhesive is being applied I prefer to drive the belt, which in Figures 3 and 4 is indicated at 28, at about 20 feet per minute in the direction shown by the arrows.

As soon as the entire belt has been coated I prefer to step the speed of the belt up to about 32 feet per minute for the application of the abrasive grains. The abrasive grains are applied by means of a nozzle indicated generally at 29, the abrasive grains being supplied from a suitable hopper through the tubes 30. Air is supplied through a tube 31 at a pressure of about 13 pounds per square inch above atmospheric pressure.

I have found that the best results are obtained if the nozzle is directed radially at a point where the belt is traveling around one of the rolls, and preferably bisects the angle between the surfaces of the belt approaching and leaving the roll. I also find that it is preferable and that the best results are obtained when the end of the nozzle is about 14 inches from the strip surface. I prefer to apply as much grain as the adhesive will hold, and therefore I prefer to let the belt make three complete revolutions. When the blast for the adhesive is shut off I apply to the surface of the belt a star roller indicated at 32 which is mounted on a pivoted arm 33. This star roller serves to pop off the excess abrasive grain.

The belt with its coating is then removed from the machine and is permitted to dry. In order to prevent the belt from drying in relatively large areas which would tend to make the belt stiff, I prefer to conduct the drying operation by hanging the belt over a slowly rotating roller, so that during the drying period the belt is simply loosely rolled along so that the adhesive bond between the coating of abrasive grains and the belt is broken up into a very large number of small bonds. Thus, the finished belt retains substantially its original flexibility and abrasive grains will not pop off when it is flexed.

I have found that with a belt made according to the procedures outlined herein the life of the belt is greatly increased, and over a period of time 30% less close down time for changing belts has been found. Since the inner surface of the belt which rides on the rollers in the grinding machine is impregnated with the elastomer, better driving friction is obtained, so that constant operating speed of the belt and higher production result. I have found that a reduction in the down time, and reduction of belt breakage whereby changing of belts in mid-coil is eliminated, results in a consistent finish from end to end of the coil. This makes the coil more saleable, as well as reducing the cost thereof. In actual production runs I have noted cost reductions as high as \$12.00 per ton when using belts according to the present invention, when compared with the use of conventional paper belts, and an average cost reduction of \$3.80 per ton has been achieved.

It will be clear that various modifications may be made without departing from the spirit of my invention, and therefore I do not intend to limit myself to all of the precise details mentioned herein. What I do claim to have invented is set forth in the claims which follow:

1. The method of making a plied endless abrasive belt, which includes the steps of preparing one ply of coating one side thereof with an elastomer, preparing at least one additional ply by impregnating the same with an elastomer, driving off the solvent in said elastomer by heating said plies to a temperature of about 200° F., softening said elastomer by heating said plies, and adhesively securing said plies together by a latex adhesive with the untreated side of said one ply on the outside, calendering said plies

and vulcanizing them under a pressure of about 2000 pounds per square inch at a temperature of about 325° F., cutting said plies to the desired belt width, applying an elastomer to the plied edges of said belt, joining the free ends of said belt with the respective ply ends in bias butting relation and with the butt joints in the respective plies in stepped relation lengthwise of said belt with the untreated side of said one ply on the outside, and vulcanizing said joint at a temperature of about 325° F., causing said belt to pass over rollers, coating said belt with an adhesive on its untreated side, and blowing abrasive grains onto said adhesive by means of a nozzle, with a pressure of about 13 pounds per square inch, the blast of said nozzle being directed substantially radially of one of said rollers, and with said nozzle being at a distance of about 14 inches from the belt surface.

2. The method of making plied endless abrasive belt, which includes the steps of preparing one ply by coating one side thereof with an elastomer, preparing at least one additional ply by impregnating the same with an elastomer, driving off the solvent in said elastomer by heating said plies to a temperature of about 200° F., softening said elastomer by heating said plies, and adhesively securing said plies together by a latex adhesive with the untreated side of said one ply on the outside, calendering said plies and vulcanizing them under a pressure of about 2000 pounds per square inch at a temperature of about 325° F., cutting said plies to the desired belt width, applying an elastomer to the plied edges of said belt, joining the free ends of said belt with the respective ply ends in bias butting relation and with the butt joints in the respective plies in stepped relation lengthwise of said belt, with the untreated side of said one ply on the outside, and vulcanizing said joint at a temperature of about 325° F., causing said belt to pass over rollers, coating said belt with an adhesive on its untreated side, blowing abrasive grains onto said adhesive by means of a nozzle, with a pressure of about 13 pounds per square inch, the blast of said nozzle being directed substantially radially of one of said rollers, and with said nozzle being at a distance of about 14 inches from the belt surface, and drying said belt by causing it to hang freely over a slowly rotating roll, whereby to break up the adhesive bond between said coating of abrasive grains and said belt into small increments.

3. The method of making an endless abrasive belt, which includes the steps of causing said belt to pass over rollers, coating said belt with an adhesive on one side, and blowing abrasive grains onto said adhesive by means of a nozzle, said nozzle being directed substantially radially of one of said rollers.

4. The method of making an endless abrasive belt, which includes the steps of causing said belt to pass over rollers, coating said belt with an adhesive on one side, and blowing abrasive grains onto said adhesive by means of a nozzle, said nozzle being directed substantially radially of one of said rollers and drying said belt by causing it to hang freely over a slowly rotating roll, whereby to break up the adhesive bond between said coating of abrasive grains and said belt into small increments.

5. The method of making an endless abrasive belt, which includes the steps of causing said belt to pass over rollers, coating said belt with an adhesive on one side, and blowing abrasive grains

onto said adhesive by means of a nozzle, with a pressure of about thirteen pounds per square inch, the blast of said nozzle being directed substantially radially of one of said rollers, and with said nozzle being at a distance of about fourteen inches from the belt surface.

6. The method of making an endless abrasive belt, which includes the steps of causing said belt to pass over rollers, coating said belt with an adhesive on one side, and blowing abrasive grains onto said adhesive by means of a nozzle, with a pressure of about thirteen pounds per square inch, the blast of said nozzle being directed substantially radially of one of said rollers, and with said nozzle being at a distance of about fourteen inches from the belt surface and drying said belt by causing it to hang freely over a slowly rotating roll, whereby to break up the adhesive bond between said coating of abrasive grains and said belt into small increments.

7. The method of making a plied endless abrasive belt, which includes the steps of impregnating a long, relatively narrow strip of textile material with an elastomer and winding it helically upon a mandrel to constitute a ply, coating said ply with a latex adhesive, adding at least one additional ply by coating another long, relatively narrow strip of textile material on one side with an elastomer and winding it helically upon said coated ply in the opposite direction and with the untreated side of said other strip outwardly, to constitute an additional ply, removing said plied belts from said mandrel, calendering said plies, and vulcanizing them.

8. The method of making a plied endless abrasive belt, which includes the steps of impregnating a long, relatively narrow strip of textile material with an elastomer and winding it helically upon a mandrel to constitute a ply, coating said ply with a latex adhesive, adding at least one additional ply by coating another long, relatively narrow strip of textile material on one side with an elastomer and winding it helically upon said coated ply in the opposite direction and with the untreated side of said other strip outwardly, to constitute an additional ply, removing said plied belts from said mandrel, calendering said plies, and vulcanizing them and slitting said plied belts into desired finished belt width.

9. The method of making a plied endless abrasive belt, which includes the steps of preparing a belt by coating one ply on one side with an elastomer, impregnating at least one additional ply with an elastomer, adhesively securing said plies together by a latex adhesive with the untreated side of the first mentioned ply on the outside, causing said belt to pass over the rollers, coating said untreated side with an adhesive, and blowing abrasive grains onto said adhesive by means of a nozzle, said nozzle being directed substantially radially of one of said rollers.

10. The method of making a plied endless abrasive belt, which includes the steps of preparing a belt by coating one ply on one side with an elastomer, impregnating at least one additional ply with an elastomer, adhesively securing said plies together by a latex adhesive with the untreated side of the first mentioned ply on the outside, causing said belt to pass over the rollers,

coating said untreated side with an adhesive, and blowing abrasive grains onto said adhesive by means of a nozzle, said nozzle being directed substantially radially of one of said rollers, and drying said belt by causing it to hang freely over a slowly rotating roll, whereby to break up the adhesive bond between said coating of abrasive grains and said belt into small increments.

11. The method of making a plied endless abrasive belt, which includes the steps of preparing a belt by coating one ply on one side with an elastomer, impregnating at least one additional ply with an elastomer, adhesively securing said plies together by a latex adhesive with the untreated side of the first mentioned ply on the outside, causing said belt to pass over rollers, coating said untreated side with an adhesive and blowing abrasive grains onto said adhesive by means of a nozzle, with a pressure of about thirteen pounds per square inch, the blast of said nozzle being directed substantially radially of one of said rollers, and with said nozzle being at a distance of about fourteen inches from the belt surface, and drying said belt by causing it to hang freely over a slowly rotating roll, whereby to break up the adhesive bond between said coating of abrasive grains and said belt into small increments.

12. The method of making a plied endless abrasive belt, which includes the steps of preparing a belt by coating one ply on one side with an elastomer, impregnating at least one additional ply with an elastomer, adhesive securing said plies together by a latex adhesive with the untreated side of the first mentioned ply on the outside, causing said belt to pass over rollers, coating said untreated side with an adhesive, and blowing abrasive grains onto said adhesive by means of a nozzle, with a pressure of about thirteen pounds per square inch, the blast of said nozzle being directed substantially radially of one of said rollers, and with said nozzle being at a distance of about fourteen inches from the belt surface.

DON S. GROVE.

#### REFERENCES CITED

The following references are of record in the file of this patent:

#### UNITED STATES PATENTS

| Number    | Name                 | Date           |
|-----------|----------------------|----------------|
| 1,929,839 | Dawson, Jr. -----    | Oct. 10, 1933  |
| 2,004,479 | Merrill -----        | June 11, 1935  |
| 2,038,782 | Ellis -----          | Apr. 28, 1936  |
| 2,059,583 | Jackson et al. ----- | Nov. 3, 1936   |
| 2,071,563 | Newcomb et al. ----- | Feb. 23, 1937  |
| 2,137,305 | Perazzoli -----      | Nov. 22, 1938  |
| 2,141,658 | Melton et al. -----  | Dec. 27, 1938  |
| 2,219,853 | Tone -----           | Oct. 29, 1940  |
| 2,226,553 | Cross -----          | Dec. 31, 1940  |
| 2,335,902 | Ball et al. -----    | Dec. 7, 1943   |
| 2,357,823 | Hatch et al. -----   | Sept. 12, 1944 |
| 2,441,970 | Lesesne -----        | May 25, 1948   |

#### FOREIGN PATENTS

| Number  | Country             | Date           |
|---------|---------------------|----------------|
| 20,668  | Great Britain ----- | Sept. 19, 1911 |
| 451,331 | Great Britain ----- | Aug. 4, 1936   |